

(No Model.)

S. A. MILLER.

COMPOSITION FOR MAKING SEWER INVERT BLOCKS.

No. 336,732.

Patented Feb. 23, 1886.

Fig. 1.

cement  
slag  
sand  
iron or steel  
sludge



Fig. 2.



WITNESSES:

Theo. G. Poston  
Jno. Mathew Ritter

INVENTOR:

S. A. Miller  
BY Munn & Co

ATTORNEYS.

Hydraulic cement.  
sand  
Iron scale or slag  
Iron or steel sludge

106 — 98

336,732

# UNITED STATES PATENT OFFICE.

SAMUEL A. MILLER, OF PHILADELPHIA, PENNSYLVANIA.

## COMPOSITION FOR MAKING SEWER INVERT-BLOCKS.

SPECIFICATION forming part of Letters Patent No. 336,732, dated February 23, 1886.

Application filed July 24, 1885. Serial No. 172,564. (No specimens.)

*To all whom it may concern:*

Be it known that I, SAMUEL A. MILLER, of Philadelphia, in the county of Philadelphia and State of Pennsylvania, have invented a 5 new and Improved Composition for Making Sewer Invert-Blocks, of which the following is a full, clear, and exact description.

The object of my invention is to provide certain new and useful improvements in the 10 method of making and in the composition of sewer invert-blocks, whereby I obtain blocks that are solid and strong, cheap and durable, and can be made easily and rapidly.

Reference is to be had to the accompanying 15 drawings, forming part of this specification, in which similar letters of reference indicate corresponding parts in all the figures.

Figure 1 is a cross-sectional elevation of my improved sewer invert-block mold and a block 20 in the same. Fig. 2 is a perspective view of my improved sewer invert-block.

The block is formed of the following composition: hydraulic cement, one part; sand, two parts; iron scale or slag, one part; iron 25 or steel sludge, one part. These ingredients are thoroughly mixed with as small a quantity

of water as possible. This composition is then filled into the mold A, the bottom block, B, of which is shaped the same as the top of the sewer invert-block, and then the composition 30 is rammed down. Before filling the mortar D into the mold I spread a thin layer, C, of a mixture of one part of sand and one part of cement on the face of the bottom block, B, of the mold. This latter mixture appears on the 35 top surface of the invert-block and gives the top a hard and smooth finish. The rest of the block is made to have great strength and durability, and to resist great pressure.

In place of the composition specified any 40 other composition of matter may be used that would produce a hard and durable article of stone.

Having thus described my invention, what I claim as new, and desire to secure by Letters 45 Patent, is—

A sewer invert-block made of artificial stone.

SAMUEL A. MILLER.

Witnesses:

DAVID S. FERGUSON,  
J. GORDON SHOWAKER.